# EUROPEAN PATENT SPECIFICATION

(11) **EP 3 291 264 B1**
(45) Date of publication and mention of the grant of the patent: **07.06.2023**
(21) Application number: 17188669.0
(22) Date of filing: 31.08.2017
(51) Int. Cl.: H01F 41/02

(54) **METHOD FOR PRODUCING SINTERED R-IRON-BORON MAGNET**
VERFAHREN ZUR HERSTELLUNG EINES GESINTERTEN R-EISEN-BOR-MAGNETS
PROCÉDÉ DE PRODUCTION D'UN AIMANT R-FER-BORE FRITTÉ

(30) Priority: 31.08.2016 CN 201610776183
(43) Date of publication of application: 07.03.2018
(73) Proprietor: Yantai Zhenghai Magnetic Material Co., Ltd., Yantai Shandong 264006 (CN)
(72) Inventor: WANG, Qingkai, Yantai, Shandong 264006 (CN); LI, Dongdong, Yantai, Shandong 264006 (CN); GENG, Guoqiang, Yantai, Shandong 264006 (CN); ZHANG, Mingjie, Yantai, Shandong 264006 (CN)
(74) Representative: Scholl, Matthias

(56) References cited:
- EP-A1- 2 555 207
- EP-A2- 3 029 689
- DE-T5-112014 003 688
- JP-A- 2015 201 546
- US-A1- 2012 139 388

## Description

The invention relates to a method for producing a sintered R-Iron-Boron (R-Fe-B) magnet and belongs to the rare earth permanent magnetic material field.

Nd-Fe-B magnets are widely used for their excellent properties. Due to the demand of the automotive and electronic fields for energy-saving motors, the sintered Nd-Fe-B magnet market will be further expanded. The improvement of the residual magnetism and coercive force of Nd-Fe-B materials is beneficial to the rapid growth of Nd-Fe-B materials in the motor market. However, the improvement of the coercive force by traditional techniques always sacrifices residual magnetism. In addition, in order to improve the coercive force, heavy rare earth elements Dy and Tb with a greater specific gravity must be used, which causes a sharp increase in magnet cost. Therefore, how to reduce the amount of heavy rare earth elements has become a hot research area in the rare earth permanent magnet field. Through analysis of magnet microstructure, grain boundary diffusion of heavy rare earth elements can effectively reduce scattered fields of grain boundaries, weaken magnetic exchange coupling, cause magnetic hardening of grain boundaries and greatly improve the coercive force in the premise that residual magnetism of magnets is not lowered basically. The improvement of magnet performance by this method can effectively control magnet costs.

The grain boundary diffusion method is to improve the coercive force of sintered Nd-Fe-B magnets and mainly diffuses the Dy or Tb element from the surface of magnets into the interior of magnets. EP 2 555 207 A1 discloses a method of producing a rare earth sintered magnet. The method includes allowing a slurry including a binder, a solvent, and a heavy rare earth compound containing a heavy rare earth element to adhere to a sintered compact of R-T-B-based rare earth magnet containing Zr; and heat treating the sintered compact. EP 3 029 689 A2 discloses a method of improving the coercive force of magnets. The method includes S2) coating a colloidal solution on the surface of a magnet and drying it; and S3) heat treating the magnet obtained in S2). In S2), the colloidal solution includes metal calcium particles; particles of a material containing a rare earth element selected from praseodymium, neodymium, gadolinium, terbium, dysprosium, holmium, erbium, thulium, ytterbium, and lutetium; and an organic solvent selected from aliphatic hydrocarbons, alicyclic hydrocarbons, alcohols, and ketones. One or more resin binders or rubber binders are dissolved in the organic solvent. In addition, US 2012/139388 A1 recites a method of producing a rare earth sintered magnet. The method includes rotating a rare earth sintered magnet body including crystal grains of (R1,R2)₂T₁₄B, in which R1 represents at least one rare earth element except for Dy and Tb, R2 represents a rare earth element including one or both of Dy and Tb, and T represents one or more transition metal elements including Fe; applying a slurry containing a compound of the rare earth element R2 to the rare earth sintered magnet body; drying the slurry while the rare earth sintered magnet body is rotated; and subjecting the rare earth sintered magnet body including the dried slurry to heat treatment. A plurality of methods has been developed for realizing grain boundary diffusion and is basically classified into two categories. One category is the evaporation process which heats and turns heavy rare earth elements into vapor and then the vapor slowly diffuses into the interior of magnets (refer to the patents CN101651038B 3/01/2007 and CN101375352A 1/12/2007). The other category is the contact process which arranges heavy rare earth elements on the surface of magnets and then enables heavy rare earth elements to penetrate grain boundaries to realize grain boundary diffusion through long-time low-temperature sintering (refer to the patents CN100565719C 2/28/2006 and CN101404195B 11/16/2007). The two processes can both realize the effect of grain boundary diffusion. The evaporation process uses parts like supports to separate magnets from heavy rare earth elements, heats and turns heavy rare earth elements into vapor which diffuses to the periphery of the magnets and then slowly into the interior of the magnets. In the evaporation process, materials which are not easy to evaporate at a high temperature are used to form a support to prevent the direct contact between magnets and heavy rare earth elements. In the actual operation process, the arrangement of the supports is relatively complicated and makes the arrangement of materials more difficult. In addition, parts like material supports occupy a larger space and greatly lower the amount of charged materials. Moreover, in order to guarantee a clean evaporation environment, parts like material supports are usually made out of materials with a low saturated vapor pressure. Therefore, the cost of processing equipment increases greatly. Moreover, as for the evaporation process, it is more difficult to control the vapor concentration. If the temperature is too low, it is difficult for heavy rare earth vapor to diffuse into the interior of magnets from the surface of magnets so that the processing time extends greatly. If the temperature is too high, the speed of producing heavy rare earth vapor in a high concentration is faster than the speed of vapor diffusing into the interior of magnets. Therefore, a layer of heavy rare earth elements forms on the surface of magnets and the effect of grain boundary diffusion cannot be realized. In the actual production process, the contact process adopts methods that realize a direct contact between heavy rare earth elements and magnets. Among the methods, the frequently-used one is the burying method which buries magnets in particles containing heavy rare earth elements. In heat treatment equipment, heavy rare earth elements diffuse into the interior of magnets from the surface of magnets through heat treatment. As for the burying method, due to the excessive contact between heavy rare earth particles and magnets, on the one hand the surface condition of magnets is damaged and on the other hand a thicker layer of heavy rare earth forms on the surface of magnets. The performance, parallelism and roughness of magnets can only be guaranteed by grinding off a lot of surface through machining. As for the other method, a heavy rare earth film is formed on the surface of magnets through sputtering and evaporation; and heavy rare earth diffuses into the interior of magnets through heat treatment in heat treatment equipment. However, due to its small treatment capacity and high treatment costs, this method is not suitable for batch production.

In view of the above-described problems, it is one objective of the invention to provide a method for producing a sintered R-iron (Fe)-boron (B) magnet.

To achieve the above objective, in accordance with one embodiment of the invention, there is provided a method for producing a sintered R-iron (Fe)-boron (B) magnet, the method comprising:
(1) producing a sintered magnet R1-Fe-B-M, wherein R1 is neodymium (Nd), praseodymium (Pr), terbium (Tb), dysprosium (Dy), gadolinium (Gd), holmium (Ho), or a combination thereof, and accounts for 27-34 wt. % of a total weight of the sintered magnet R1-Fe-B-M, the boron (B) accounts for 0.8-1.3 wt. % of the total weight of the sintered magnet R1-Fe-B-M; M is titanium (Ti), vanadium (V), chromium (Cr), manganese (Mn), cobalt (Co), gallium (Ga), copper (Cu), silicon (Si), aluminum (Al), zirconium (Zr), niobium (Nb), tungsten (W), molybdenum (Mo), or a combination thereof, and accounts for 0-5 wt. % of the total weight of the sintered magnet R1-Fe-B-M; and the rest is Fe;
(2) washing the sintered magnet using an acid solution and deionized water, successively, and drying the sintered magnet to yield a treated magnet;
(3) mixing a heavy rare earth element powder RX, an organic solid powder EP and an organic solvent ET to yield a slurry RXE, coating the slurry RXE on a surface of the treated magnet, and drying the treated magnet to yield a treatment unit comprising an RXE layer, wherein the heavy rare earth element powder RX is Dy powder, Tb powder, or a combination thereof, the organic solid powder EP is rosin-modified alkyd resin, thermoplastic phenolic resin, urea-formaldehyde resin, or a combination thereof, and the organic solvent ET is ethyl alcohol, ether, benzene, glycerol, ethanediol, or a combination thereof; and
(4) heating the treatment unit in (3) at a temperature of between 850°C and 970°C for between 0.5 and 48 hrs, quenching the treatment unit, and then aging the treatment unit at a temperature of between 430°C and 650°C for between 2 and 10 hrs.

The innovation of the invention is that: the heavy rare earth element powder RX, the organic solid EP and the organic solvent ET are used to prepare the slurry RXE; the evenly stirred slurry RXE is coated on the surface of the treated magnet; after drying treatment, an RXE layer is formed on the surface of the magnet to realize the effect of arranging heavy rare earth elements on the surface of the magnet. The RXE layer can be arranged on the surface of the magnet through brush coating, dipping, roller coating and spray painting. The RXE layer is highly controllable in thickness and uniformity, is not easy to fall off and is easy to realize batch production. Since the heavy rare earth element RX is wrapped by the organic solid powder EP after drying treatment, the RXE layer on the surface of the magnet is not easy to oxidize. Therefore, the magnet can keep stable in the air for a long time. During heat treatment, the organic solid powder EP and the organic solvent ET are separated from the magnet so the content of carbon in the magnet will not increase significantly.

In a class of this embodiment, in step (3), the slurry RXE needs to be stirred in use. Since the density of the powder RX is much greater than that of EP and ET, the slurry RXE still cannot keep stable and uniform for a long time although the organic solid EP used in the thick liquid prevents the powder RXfrom settling obviously. Therefore, the slurry RXE is stirred preferably in use.

In a class of this embodiment, in (3), the weight percent of the RX in the slurry RXE ranges from 30 wt. % to 90 wt. %. When the weight percent of the RX in the slurry RXE is too low, since the density of the powder RX is higher, the distribution uniformity of the RX in the slurry RXE lowers even if stir treatment is carried out so that the RX on the surface of the treated magnet is not even in distribution. When the weight percent of the RX in the slurry RXE is too high, the flowability of the thick liquid becomes lower and the viscosity of the thick liquid becomes higher so it is not easy to arrange an RXE layer which is even in thickness on the surface of the treated magnet.

In a class of this embodiment, in step (3), the slurry RXE is arranged on the surface of a regular square magnet through brush coating and roller coating. The slurry RXE is arranged on the surface of an irregular magnet through dipping and spray coating.

As for a regular square magnet, the slurry RXE forms an RXE layer which is even in thickness on the surface of the magnet through brush coating, roller coating, dipping and spray coating. The powder RX is distributed on the surface of the magnet evenly. As for an irregular magnet, it is easier to adopt dipping and spray coating to realize the even distribution of the RXE layer.

In a class of this embodiment, in step (3), the grain size of the heave rare earth powder RX is less than 30µm and the thickness of the RXE layer ranges from 10µm to 200µm. When the grain size of RX particles is greater than 30µm, it is easy for RX to settle and not easy to form the slurry RXE with high uniformity. Therefore, it is harder to form an RXE layer on the surface of the magnet. When the coating is thinner it is easy to form granular bulges on the coating surface and then the diffusion uniformity of the magnet will finally be affected. The thickness of the RXE layer is controlled within a certain range because when the RXE layer is too thin the grain size of the RX particles in the RXE layer is close to the thickness of the coating and it is harder to realize even distribution of the RX particles. Therefore, the heavy rare earth elements which diffuse into the interior of the magnet from the surface of the magnet are not even in distribution, and finally the uniformity of the magnet is poor. When the RXE layer is too thick, the RXE layer has excessive RX. The excessive RX cannot entirely diffuse into the interior of the magnet during heat treatment, gathers on the surface of the magnet, corrodes the surface of the magnet, and affects the surface condition of the magnet. When the RXE layer is too thick, the RXE layer has excessive EP and ET. Therefore, a lot of organic materials come out during heat treatment. If the excessive EP and ET cannot be discharged in time, the air of heat treatment equipment will be affected, the content of carbon and oxygen in the magnet will increase and the magnet performance will be finally affected.

In step (3), the organic solvent ET is one or more of ethanol, benzene, glycerol and ethanediol and the ethanol is the preferred one. Compared to ethanol, benzene, glycerol and ethanediol are more harmful to human bodies. During solidification and heat treatment, a lot of ET will fall off at a high temperature. If benzene, glycerol and ethanediol are used as an organic solvent ET, they have higher requirements on the air tightness, air-discharging capacity and safety of equipment. Therefore, the cost of equipment increases.

In a class of this embodiment, in step (3), the treated magnet at least has one direction with thickness less than 10 mm.

During heat treatment, the heavy rare earth element RX diffuses into the interior of the magnet through liquid-like grain boundaries. The diffusion is mainly driven by concentration differences. If the concentration difference is lower, the driving force is not strong and then the diffusion is slow. When the magnet thickness is greater than 10 mm, it is very hard to realize full diffusion, and then the magnetic properties like Hk/Hcj become poor, and finally the temperature resistance of the magnet is affected.

The invention uses the heavy rare earth element powder RX, organic solid EP and organic solvent ET to prepare slurry RXE which is arranged on the surface of the magnet. After drying treatment, an RXE layer is formed on the surface of the magnet to realize the arrangement of heavy rare earth elements on the surface of the magnet, and then the magnet can be stored stably in the air for a long time. During heat treatment, the organic solid powder EP and the organic solvent ET are separated from the magnet so the content of carbon in the magnet will not increase obviously. The heavy rare earth elements in the heavy rare earth element powder RX diffuse into the interior of the magnet and realize grain boundary diffusion to improve magnet properties. During batch production, the slurry RXE can be arranged on the surface of the magnet through brush coating, dipping, roller coating and spray coating. The thickness of the RXE layer is controllable. It is easy to realize automatic production. The invention is slightly affected by magnet shapes.

For further illustrating the invention, experiments detailing a method for producing a sintered R-Fe-B magnet are described hereinbelow combined with the drawings. It should be noted that the following examples are intended to describe and not to limit the invention.

### Example 1

Raw materials were melted in a vacuum melting furnace under the protection of inert gas to form R-Fe-B alloy scales with the thickness ranging from 0.1 mm to 0.5 mm. The metallographic grain boundaries of the scales were clear. After mechanical comminution and hydro-treatment, the alloy scales were ground by nitrogen gas flow until the surface mean diameter (SMD) was 3.2 µm. The 1.19×10⁶ A/m (15 kOe) magnetic field orientation was adopted for compression molding to produce pressings. The density of the pressings was 3.95 g/cm³. The pressings were sintered in a vacuum in a sintering furnace. The pressings were sintered at the highest temperature of 1080°C for 330 minutes to produce green pressings. After wire-electrode cutting, the green pressings become magnetic sheets. The size of the magnetic sheets was 40 mm*30 mm*2.1 mm and the size tolerance was ±0.03 mm. The surface of the magnetic sheets was washed by acid solutions and deionized water. After drying treatment, a treated magnet M1 was produced. The composition of the treated magnet M1 is shown in Table 2 below.

Heavy rare earth element powder TbH, organic solid rosin-modified alkyd resin powder and ethanol were mixed to prepare a slurry RXE. The weight percents of the TbH, the rosin-modified alkyd resin powder and the ethanol were 60 wt. %, 5 wt. % and 35 wt. %, respectively. Stir the slurry RXE for about 60 minutes. Dip the treated magnet M1 in the slurry RXE for about 3 seconds and then take the treated magnet M1 out. Put the treated magnet M1 in a drying oven at a temperature of 70°C for about 15 minutes to produce the treated magnet with an RXE layer on the surface.

Put the treated magnet with an RXE layer in a material box for heat treatment in heat treatment equipment. After the temperature rose to 920°C, keep the magnet at the temperature of 920°C for 18 hours and then chill the magnet quickly. Then, the temperature rose to 500°C for aging treatment (the aging treatment refers to the heat treatment process that the properties, shapes and sizes of alloy work pieces after solution treatment, cold plastic deformation or casting and forging change with time at a higher temperature or the room temperature). Keep the magnet at a temperature of 500°C for 4 hours and then chill the magnet quickly to the room temperature to produce the magnet M2.

**Table 1 Comparison of properties of magnet M2 and treated magnet M1 before diffusion treatment**

| Items | Density | Br | Hcj | (BH) max | Hk/Hcj |
|---|---|---|---|---|---|
| M2 | 7.56 g/cm³ | 1.39 T (13.87 kGs) | 1.81×10⁶ A/m (22.79 kOe) | 368.8 kJ/m³ (46.35 MGOe) | 0.95 |
| M1 | 7.56 g/cm³ | 1.41 T (14.06 kGs) | 1.07×10⁶ A/m (13.46 kOe) | 374.7 kJ/m³ (47.09 MGOe) | 0.97 |

**Table 2 Comparison of main compositions of magnet M2 and treated magnet M1 before diffusion treatment**

| Items | B | Al | Co | Dy | Tb | Pr | Nd |
|---|---|---|---|---|---|---|---|
| M2 measured value % | 0.97 | 0.1 | 0.89 | 0.51 | 0.48 | 4.71 | 25.65 |
| M1 measured value % | 0.97 | 0.1 | 0.9 | 0.52 | 0 | 4.72 | 25.67 |

As shown in Tables **1** and **2,** compared to the treated magnet M1, the residual magnetism Br of the magnet M2 is reduced by about 0.019 T (190Gs), and the Hcj of the magnet M2 increases by about 7.42×10⁵A/m (9.33 kOe) through this method. According to the composition tests, compared to the treated magnet M1, Tb of the magnet M2 increases by about 0.48 wt. %.

**Table 3 Comparison of CSON element content between magnet M2 and treated magnet M1 before diffusion treatment**

| Items | C | S% | O% | N% |
|---|---|---|---|---|
| M2 measured value % | 0.0742 | 0.0011 | 0.0999 | 0.0304 |
| M1 measured value % | 0.0721 | 0.0009 | 0.0980 | 0.0321 |

Table **3** shows the comparison of the CSON element content of the magnet before and after diffusion treatment. The content of C and the content of O both do not have an obvious increase. It means that most organic rosin-modified alkyd resin does not diffuse into the interior of the magnet during the diffusion process.

### Example 2

Raw materials were melted in a vacuum melting furnace under the protection of inert gas to form R-Fe-B alloy scales with the thickness ranging from 0.1 mm to 0.5 mm. The metallographic grain boundaries of the scales were clear. After mechanical comminution and hydro-treatment, the alloy scales were ground by nitrogen gas flow until the surface mean diameter (SMD) was 3.1 µm. The 1.19×10⁶ Aim (15 kOe) magnetic field orientation was adopted for compression molding to produce pressings. The density of the pressings was 3.95 g/cm³. The pressings were sintered in a vacuum in a sintering furnace. The pressings were sintered at the highest temperature of 1085°C for 330 minutes to produce green pressings. After wire-electrode cutting, the green pressings become magnetic sheets. The size of the magnetic sheets was 40 mm*30 mm*3 mm and the size tolerance was ±0.03 mm. The surface of the magnetic sheets was washed by acid solutions and deionized water. After drying treatment, a treated magnet M3 was produced. The composition of the treated magnet M3 is shown in Table **5** below.

Heavy rare earth element powder TbF, polyvinyl butyral and ethanol were mixed to prepare a slurry RXE. The weight percents of the TbF, the polyvinyl butyral and the ethanol were 65 wt. %, 6 wt. % and 29 wt. %, respectively. Stir the slurry RXE for about 60 minutes. Dip the treated magnet M3 in the slurry RXE for about 3 seconds and then take the treated magnet M3 out. Put the treated magnet M3 in a drying oven at a temperature of 70°C for about 15 minutes to produce the treated magnet with an RXE layer on the surface.

Put the treated magnet with an RXE layer in a material box for heat treatment in heat treatment equipment. After the temperature rose to 920°C, keep the magnet at the temperature of 930°C for 20 hours and then chill the magnet quickly. Then, the temperature rose to 520°C for aging treatment. Keep the magnet at a temperature of 520°C for 4 hours and then chill the magnet quickly to the room temperature to produce the magnet M4.

**Table 4 Comparison of properties of magnet M4 and treated magnet M3 before diffusion treatment**

| Items | Density | Br | Hcj | (BH) max | Hk/Hcj |
|---|---|---|---|---|---|
| M4 | 7.56 g/cm³ | 1.42 T (14.19 kGs) | 1.94×10⁶ Aim (24.32 kOe) | 384.0 kJ/m³ (48.25 MGOe) | 0.95 |
| M3 | 7.56 g/cm³ | 1.44 T (14.36 kGs) | 1.15×10⁶ A/m (14.46 kOe) | 390.6 kJ/m³ (49.09 MGOe) | 0.97 |

**Table 5 Comparison of main compositions of magnet M4 and treated magnet M3 before diffusion treatment**

| Items | B | Al | Co | Tb | Pr | Nd |
|---|---|---|---|---|---|---|
| M4 measured value % | 0.97 | 0.15 | 0.8 | 0.92 | 4.72 | 25.63 |
| M3 measured value % | 0.97 | 0.15 | 0.8 | 0.5 | 4.72 | 25.67 |

As shown in Tables **4** and **5,** compared to the treated magnet M3, the residual magnetism Br of the magnet M4 is reduced by about 0.017 T (170Gs), and the Hcj of the magnet M4 increases by about 7.85×10⁵A/m (9.86 kOe) through this method. According to the composition tests, compared to the treated magnet M3, Tb of the magnet M4 increases by about 0.48 wt. %.

**Table 6 Comparison of CSON element content between magnet M4 and treated magnet M3 before diffusion treatment**

| Items | C | S% | O% | N% |
|---|---|---|---|---|
| M4 measured value % | 0.0721 | 0.0014 | 0.0673 | 0.0312 |
| M3 measured value % | 0.0678 | 0.0012 | 0.0636 | 0.0298 |

Table **6** shows the comparison of the CSON element content of the magnet before and after diffusion treatment. The content of C and the content of O both do not have an obvious increase. It means that most polyvinyl butyral does not diffuse into the interior of the magnet during the diffusion process.

### Example 3

Raw materials were melted in a vacuum melting furnace under the protection of inert gas to form R-Fe-B alloy scales with the thickness ranging from 0.1 mm to 0.5 mm. The metallographic grain boundaries of the scales were clear. The alloy scales were ground by jet milling to yield powders having the surface mean diameter (SMD) of 3.2 µm. The 1.19×10⁶ Aim (15 kOe) magnetic field orientation was adopted for compression molding to produce pressings. The density of the pressings was 3.95 g/cm³. The pressings were sintered in a vacuum in a sintering furnace. The pressings were sintered at the highest temperature of 1085°C for 300 minutes to produce green pressings. After wire-electrode cutting, the green pressings become magnetic sheets. The size of the magnetic sheets was 40 mm*25 mm*4.5 mm and the size tolerance was ±0.03 mm. The surface of the magnetic sheets was washed by acid solutions and deionized water. After drying treatment, a treated magnet M5 was produced. The composition of the treated magnet M5 is shown in Table **8** below.

Heavy rare earth element powders TbF and Tb, organic solid urea resin and ethanol were mixed to prepare a slurry RXE, and the weight percents thereof were 60 wt. %, 6 wt. % and 34 wt. %, respectively. The maximum particle size of the mixed powders of TbF and Tb was less than 18 µm. Stir the slurry RXE for about 60 minutes. The treated magnet M5 was coated with a layer of RXE slurry. Put the treated magnet M5 in a drying oven at a temperature of 90°C for about 15 minutes to produce the treated magnet with an RXE layer on the surface. The weight of the treated magnet M5 was increased by 1.02 wt. %.

Put the treated magnet with an RXE layer in a material box for heat treatment in heat treatment equipment. After the temperature rose to 930°C, keep the magnet at the temperature of 930°C for 25 hours and then chill the magnet quickly. Then, the temperature rose to 540°C for aging treatment. Keep the magnet at a temperature of 540°C for 4 hours and then chill the magnet quickly to the room temperature to produce the magnet M6.

**Table 7 Comparison of properties of magnet M6 and treated magnet M5 before diffusion treatment**

| Items | Density | Br | Hcj | (BH)max | Hk/Hcj |
|---|---|---|---|---|---|
| M6 | 7.58 g/cm³ | 1.42 T (14.16 kGs) | 2.01×10⁶ A/m (25.22 kOe) | 380.9 kJ/m³ (47.87 MGOe) | 0.94 |
| M5 | 7.57 g/cm³ | 1.43 T (14.31 kGs) | 1.23×10⁶ A/m (15.42 kOe) | 387.8 kJ/m³ (48.73 MGOe) | 0.98 |

**Table 8 Comparison of main compositions of magnet M6 and treated magnet M5 before diffusion treatment**

| Items | B | Al | Co | Dy | Tb | Pr | Nd |
|---|---|---|---|---|---|---|---|
| M6 measured value % | 0.98 | 0.1 | 0.6 | 0.68 | 0.91 | 5.87 | 22.37 |
| M5 measured value % | 0.99 | 0.1 | 0.6 | 0.70 | 0.5 | 5.88 | 22.40 |

As shown in Tables **7** and **8,** compared to the treated magnet M5, the residual magnetism Br of the magnet M6 is reduced by about 0.015 T (150 Gs), and the Hcj of the magnet M6 increases by about 7.80×10⁵ A/m (9.8 kOe) through this method. According to the composition tests, compared to the treated magnet M5, Tb of the magnet M6 increases by about 0.41 wt. %. Since the magnet is relatively thick, the holding time for thermal treatment at 930°C is significantly longer than that in examples 1 and 2.

**Table 9 Comparison of CSON element content between magnet M6 and treated magnet M5 before diffusion treatment**

| Items | C | S% | O% | N% |
|---|---|---|---|---|
| M6 measured value % | 0. 0873 | 0. 0017 | 0.0883 | 0. 0334 |
| M5 measured value % | 0.0798 | 0. 0019 | 0.0857 | 0. 0301 |

Table **9** shows the comparison of the CSON element content of the magnet before and after diffusion treatment. The content of C and the content of O both do not have an obvious increase. It means that most urea resin does not diffuse into the interior of the magnet during the diffusion process.

## Claims

1. A method for producing a sintered magnet, the method consisting of:
(1) producing a sintered magnet R1-Fe-B-M, wherein R1 is neodymium (Nd), praseodymium (Pr), terbium (Tb), dysprosium (Dy), gadolinium (Gd), holmium (Ho), or a combination thereof, and accounts for 27-34 wt. % of a total weight of the sintered magnet R1-Fe-B-M; the boron (B) accounts for 0.8-1.3 wt. % of the total weight of the sintered magnet R1-Fe-B-M; M is titanium (Ti), vanadium (V), chromium (Cr), manganese (Mn), cobalt (Co), gallium (Ga), copper (Cu), silicon (Si), aluminum (Al), zirconium (Zr), niobium (Nb), tungsten (W), molybdenum (Mo), or a combination thereof, and accounts for 0-5 wt. % of the total weight of the sintered magnet R1-Fe-B-M; and the rest is Fe;
(2) washing the sintered magnet using an acid solution and deionized water, successively, and drying the sintered magnet to yield a treated magnet;
(3) mixing a heavy rare earth element powder RX, an organic solid powder EP and an organic solvent ETto yield a slurry RXE, coating the slurry RXE on a surface of the treated magnet, and drying the treated magnet to yield a treatment unit comprising an RXE layer, wherein the organic solvent ET is ether, benzene, ethyl alcohol, glycerol, ethanediol, or a combination thereof; and
(4) heating the treatment unit in (3) at a temperature of between 850°C and 970°C for between 0.5 and 48 hrs, quenching the treatment unit, and then aging the treatment unit at a temperature of between 430°C and 650°C for between 2 and 10 hrs;
**characterized in that** in (3), the heavy rare earth element powder RX is Dy powder, Tb powder, or a combination thereof; and the organic solid powder EP is a rosin-modified alkyd resin, a thermoplastic phenolic resin, an urea-formaldehyde resin, or a combination thereof.

2. The method of claim 1, **characterized in that** a particle size of the heavy rare earth element powder RX is less than 100 µm.

3. The method of claim 1, **characterized in that** in (3), the RXE layer is between 3 and 500 µm in thickness.

4. The method of claim 1, **characterized in that** in (3), a weight percent of the powder RX in the slurry RXE ranges from 30 wt. % to 90 wt. %.

5. The method of claim 1, **characterized in that** in (3), a thickness of the treated magnet in at least one direction is less than 10 mm.

6. The method of claim 2, **characterized in that** the particle size of the heavy rare earth element powder RX is less than 30 µm.

7. The method of claim 3, **characterized in that** the RXE layer is between 10 and 200 µm in thickness.

## Patentansprüche

1. Verfahren zur Herstellung eines gesinterten Magneten, wobei das Verfahren aus Folgendem besteht:
(1) Herstellen eines gesinterten Magneten R1-Fe-B-M, wobei R1 Neodym (Nd), Praseodym (Pr), Terbium (Tb), Dysprosium (Dy), Gadolinium (Gd), Holmium (Ho) oder eine Kombination davon ist und 27-34 Gew.-% eines Gesamtgewichts des gesinterten Magneten R1-Fe-B-M ausmacht; das Bor (B) 0,8-1,3 Gew.-% des Gesamtgewichts des gesinterten Magneten R1-Fe-B-M ausmacht; M Titan (Ti), Vanadium (V), Chrom (Cr), Mangan (Mn), Kobalt (Co), Gallium (Ga), Kupfer (Cu), Silizium (Si), Aluminium (Al), Zirkonium (Zr), Niob (Nb), Wolfram (W), Molybdän (Mo) oder eine Kombination davon ist und 0-5 Gew.-% des Gesamtgewichts des gesinterten Magneten R1-Fe-B-M ausmacht; und der Rest Fe ist;
(2) Waschen des gesinterten Magneten unter Verwendung einer Säurelösung und von entionisiertem Wasser nacheinander und Trocknen des gesinterten Magneten, um einen behandelten Magneten zu ergeben;
(3) Mischen eines schweren Seltenerdelementpulvers RX, eines organischen Feststoffpulvers EP und eines organischen Lösungsmittels ET, um eine Aufschlämmung RXE zu ergeben, Auftragen der Aufschlämmung RXE auf einer Oberfläche des behandelten Magneten und Trocknen des behandelten Magneten, um eine Behandlungseinheit zu ergeben, die eine RXE-Schicht umfasst, wobei das organische Lösungsmittel ET Ether, Benzol, Ethylalkohol, Glycerin, Ethandiol oder eine Kombination davon ist; und
(4) Erhitzen der Behandlungseinheit in (3) bei einer Temperatur zwischen 850 °C und 970 °C für zwischen 0,5 und 48 Std., Abschrecken der Behandlungseinheit und dann Altern der Behandlungseinheit bei einer Temperatur zwischen 430 °C und 650 °C für zwischen 2 und 10 Std.;
**dadurch gekennzeichnet, dass** in (3) das schwere Seltenerdelementpulver RX Dy-Pulver, Tb-Pulver oder eine Kombination davon ist; und das organische Feststoffpulver EP ein Kolophonium-modifiziertes Alkydharz, ein thermoplastisches Phenolharz, ein Harnstoff Formaldehyd-Harz oder eine Kombination davon ist.

2. Verfahren nach Anspruch 1, **dadurch gekennzeichnet, dass** eine Partikelgröße des schweren Seltenerdelementpulvers RX weniger als 100 µm ist.

3. Verfahren nach Anspruch 1, **dadurch gekennzeichnet, dass** in (3) die RXE-Schicht zwischen 3 und 500 µm dick ist.

4. Verfahren nach Anspruch 1, **dadurch gekennzeichnet, dass** in (3) ein Gewichtsprozent des Pulvers RX in der Aufschlämmung RXE von 30 Gew.-% bis 90 Gew.-% reicht.

5. Verfahren nach Anspruch 1, **dadurch gekennzeichnet, dass** in (3) eine Dicke des behandelten Magneten in zumindest einer Richtung weniger als 10 mm ist.

6. Verfahren nach Anspruch 2, **dadurch gekennzeichnet, dass** die Partikelgröße des schweren Seltenerdelementpulvers RX weniger als 30 µm ist.

7. Verfahren nach Anspruch 3, **dadurch gekennzeichnet, dass** die RXE-Schicht zwischen 10 und 200 µm dick ist.

## Revendications

1. Procédé de production d'un aimant fritté, le procédé consistant en :
(1) la production d'un aimant fritté R1-Fe-B-M, dans lequel R1 est le néodyme (Nd), le praséodyme (Pr), le terbium (Tb), le dysprosium (Dy), le gadolinium (Gd), l'holmium (Ho) ou une combinaison de ceux-ci, et représente 27 à 34 % en poids du poids total de l'aimant fritté R1-Fe-B-M ; le bore (B) représente 0,8 à 1,3 % en poids du poids total de l'aimant fritté R1-Fe-B-M ; M est le titane (Ti), le vanadium (V), le chrome (Cr), le manganèse (Mn), le cobalt (Co), le gallium (Ga), le cuivre (Cu), le silicium (Si), l'aluminium (Al), le zirconium (Zr), le niobium (Nb), le tungstène (W), le molybdène (Mo) ou une combinaison de ceux-ci, et représente 0 à 5 % en poids du poids total de l'aimant fritté R1-Fe-B-M ; et le reste représente Fe ;
(2) le lavage de l'aimant fritté en utilisant successivement une solution acide et de l'eau désionisée et le séchage de l'aimant fritté pour produire un aimant traité ;
(3) le mélange d'une poudre d'élément de terre rare lourd RX, d'une poudre organique solide EP et d'un solvant organique ET pour produire une pâte RXE, l'enduction de la pâte RXE sur une surface de l'aimant traité, et le séchage de l'aimant traité pour produire une unité de traitement comprenant une couche de RXE, ledit solvant organique ET étant l'éther, le benzène, l'alcool éthylique, le glycérol, l'éthanediol ou une combinaison de ceux-ci ; et
(4) le chauffage de l'unité de traitement en (3) à une température comprise entre 850°C et 970°C pendant une durée comprise entre 0,5 et 48 heures, la trempe de l'unité de traitement et ensuite le vieillissement de l'unité de traitement à une température comprise entre 430°C et 650°C pendant une durée comprise entre 2 et 10 heures ;
**caractérisé en ce qu'**en (3), la poudre d'élément de terre rare lourd RX est une poudre de Dy, une poudre de Tb ou une combinaison de celles-ci ; et la poudre solide organique EP est une résine d'alkyde modifiée par de la colophane, une résine phénolique thermoplastique, une résine d'urée-formaldéhyde ou une combinaison de celles-ci.

2. Procédé selon la revendication 1, **caractérisé en ce qu'**une taille de particule de la poudre d'élément de terre rare lourd RX est inférieure à 100 µm.

3. Procédé selon la revendication 1, **caractérisé en ce qu'**en (3), la couche de RXE fait entre 3 et 500 µm d'épaisseur.

4. Procédé selon la revendication 1, **caractérisé en ce qu'**en (3), un pourcentage en poids de la poudre RX dans la pâte RXE va de 30 % en poids à 90 % en poids.

5. Procédé selon la revendication 1, **caractérisé en ce qu'**en (3), une épaisseur de l'aimant traité dans au moins une direction est inférieure à 10 mm.

6. Procédé selon la revendication 2, **caractérisé en ce que** la taille de particule de la poudre d'élément de terre rare RX est inférieure à 30 µm.

7. Procédé selon la revendication 3, **caractérisé en ce que** la couche de RXE fait entre 10 et 200 µm d'épaisseur.
